# EUROPEAN PATENT SPECIFICATION

(11) **EP 0 037 724 B1**
(45) Date of publication and mention of the grant of the patent: **22.06.1983**
(21) Application number: 81301461.0
(22) Date of filing: 03.04.1981
(51) Int. Cl.: G03C 5/54, C08L 53/00

(54) **Photographic colour diffusion transfer materials containing timing layers**
Verzögerungsschichten enthaltende photographische Diffusionsfarbaufzeichnungsmaterialien
Matériaux photographiques de diffusion des couleurs par transfert comportant des couches retardatrices

(30) Priority: 03.04.1980 GB 8011387
(43) Date of publication of application: 14.10.1981
(73) Proprietor: EASTMAN KODAK COMPANY (a New Jersey corporation), Rochester, New York 14650 (US); KODAK LIMITED, Hemel Hempstead, Hertfordshire HP1 1JU (GB)
(72) Inventor: Schofield, Edward, Chesham Buckinghamshire HP5 2BP (GB); Wagner, Hans Max, Stanmore Middlesex HA7 4SH (GB)
(74) Representative: Pepper, John Herbert

## Description

This invention relates to photographic colour diffusion transfer materials.

It is customary in many photographic colour diffusion transfer materials to incorporate an acid substance which will cause a lowering of the pH when processing is completed. However, without any special arrangements such a lowering of the pH could occur too rapidly and before processing was complete. Such a difficulty has been overcome by having a timing layer between the acid layer and the point of discharge of the alkaline processing composition. The timing layer only allows passage of the alkali after a given time thus giving greater control in the design of the photographic material.

British Specification 1,544,306 describes timing layers comprising a film-forming linear polymer with a molecular weight of from 5000 to 100,000 wherein the linear chain of the polymer comprises alternating hydrophilic and hydrophobic segments joined to one another through carbonate, urethane and/or ester groups. While it is suggested that the hydrophobic segments could be polymeric, the specific polymers disclosed employ only monomeric hydrophobic groups. The polymers employed are contrasted with prior art vinyl polymers wherein the polymer backbone consists of carbon only and it is suggested that such polymers are inferior as timing layers to those having heteroatoms in their backbone.

Since the development process is temperature-dependent, it is often necessary to adjust the temperature-dependence of the timing layer to obtain maximum temperature latitude of processing.

The present invention provides addition block co-polymer timing layers whose break-down time varies with changes in temperature and thus enables temperature dependence profiles to be matched to the requirements of a particular image transfer material.

According to the present invention there is provided a photographic colour diffusion transfer material containing an acid layer and a timing layer characterised in that the timing layer comprises an addition block copolymer comprising blocks of polymerised styrene or a substituted styrene and blocks of a homo- or co-polymer which is alkali-permeable or which becomes alkali-permeable after contact with alkali.

It is believed that the block copolymers employed herein have the ability to separate into micro- phases due to the incompatability of their constituent parts. It is thought therefore that the timing layer made therefrom can be considered as a hydrophilic or potentially hydrophilic matrix containing hydrophobic regions. The morphology of the layer can be controlled by varying the lengths and the ratio of the hydrophobic and hydrophilic blocks. Such variations, in turn, cause the break-down time behaviour to vary.

The polymerised styrene blocks may be formed from styrene itself or styrene substituted with, for example, hydrocarbon groups, particularly alkyl groups of 1-4 carbon atoms. Specific substituted styrenes include p-methylstyrene and a-methylstyrene.

The monomers from which the alkali-permeable blocks are made may vary widely. The monomers may, for example, contain acid groups or basic nitrogen-containing groups. Alternatively they may contain hydrolysable groups, for example, esters. Particular examples of such monomers are vinyl acetate, N-vinylcarpolactam, N-vinylpyrrolidone, hydroxyethyl methacrylate, methacrylic acid and N-vinylimidazole either alone or in combination.

The block copolymer may contain 10--45 weight percent styrene blocks, preferably 15-20 weight percent.

The block copolymers may be prepared by known methods, for example that described by T. Otsu, J. Polym. Sci. 26 236 (1957) but any other method suitable for preparing block copolymers described in the literature can be used. e.g. described for example in Block and Graft Copolymerization by R.J. Ceresa, Wiley, London 1973.

The present timing layers may be present in complete dye diffusion transfer film units or in separate photosensitive materials or receiving sheets.

Various formats for colour diffusion transfer film units are described in the prior art, such as U.S. Patents 3,415,644, 3,415,645, 3,415,646, 3,647,437, 3,636,707 and 3,756,815 and Canadian Patents 928,559 and 674,082. In these formats, the image-receiving layer containing the photographic image for viewing can remain permanently attached and integral with the image-generating and auxiliary layers present in the structure when a transparent support is employed on the viewing side of the film unit.

Other so-called "peel-apart" formats for colour diffusion transfer film units are described, for example, in U.S. Patents 2,983,606, 3,362,819 and 3,362,821. In those formats, an image-receiving element is separated from the photosensitive element after development and transfer of the dyes to the image-receiving layer.

A preferred format of the colour transfer film units of this invention is depicted in British Specifications 1,330,524 and 1,405,662 which describe integral colour transfer formats consisting of a laminated sandwich of an integral-negative-receiver element, a transparent processing cover sheet and, adapted to be spaced between them, an opaque viscous processing composition spread by rupturing a pod by drawing the transfer sandwich between a pair of juxtaposed rollers. On the transparent film support of the integral-negative-receiver are coated successively an image-receiving layer, a white reflective pigment layer, an opaque layer, three image-forming units and an overcoat layer. On the transparent film support of the cover sheet are coated successively a neutralizing layer and a timing layer. The unit is exposed through the cover sheet while the viewing of the image is from the opposite side.

Cover sheets useful for the above format, as well as for all other colour transfer systems, are described in British Patents 878,064 and 1,340,349 and U.S. Patent 3,414,411.

Other film unit formats in which this invention may be employed are described in U.S. Patents 3,362,821, 3,415,644, 3,415,645, 3,415,646, 3,647,437, 3,635,707 and 3,362,819 and British Specification 1,330,524.

The dye image-providing materials which may be employed in this invention generally may be characterized as either (1) initially soluble or diffusible in the processing composition but being selectively rendered nondiffusible in an imagewise pattern as a function of development, such as those disclosed, for example, in U.S. Patents 2,647,049, 2,661,293, 2,698,244, 2,698,798, 2,802,735, 2,774,668 and 2,983,606 or (2) initially insoluble or nondiffusible in the processing composition but being selectively rendered diffusible in an imagewise pattern as a function of development, for example, those disclosed, for example, in U.S. Patents 3,227,550, 3,227,551, 3,227,552, 3,227,554, 3,243,294 and 3,445,228. These materials may be preformed dyes or dye precursors, e.g. colour couplers or oxichromic compounds.

In a preferred embodiment of this invention, the dye image-providing material is a nondiffusible redox dye releaser. Such compounds are, generally speaking, compounds which can be oxidized by oxidized developing agent, i.e., crossoxidized, to provide a species which will release a diffusible dye, such as by alkaline hydrolysis. Such redox dye releasers are described in U.S. Patents 3,725,062, 3,698,897, 3,628,952, 3,443,939, 3,443,940, 3,928,312, 3,929,760, 3,980,379, 3,993,638, 3,954,476, 3,932,380 and U.S. Published Patent Application B-351,673, British Specifications 1,405,662, 1,464,104, 1,464,105, 1,458,471, 1,465,183 and 1,465,184.

The following Examples are included for a better understanding of the invention.

### Examples 1-5

### Preparation of polystyrene with diethyldithiocarbamate end groups (T-PST)

Styrene (60 cm³), purified in the usual manner, and tetraethylthiuram disulphide (0.6 g) were heated together at 80°C under nitrogen for 7 hours. The mixture was diluted with toluene; the polymer was precipitated from the solution into ethanol, twice further reprecipitated from toluene into ethanol and dried at room temperature under vacuum. Yield 18.8 g of white powder.
Analysis: C: 91.76; H: 7.86; N: 0.16; S: 0.7.

### Preparation of poly(styrene)-b-(vinyl acetate)

Vinyl acetate (VAcO), T-PST (prepared above) and optionally benzene (see Table I for details) were mixed in a glass vacuum ampoule, degassed by successive freeze-thaw cycles and sealed under vacuum. The mixture was irradiated using a high pressure mercury lamp, precipitated into petroleum spirit, filtered and dried under vacuum. Polystyrene and poly(vinyl acetate) homopolymer were removed by extraction with boiling cyclohexane and methanol respectively. The reaction conditions and yields are shown in Table I. The molar ratio of the two units in the block copolymer were determined by nmr and are also listed in Table I.

The reaction has also been shown to work perfectly well under a blanket of nitrogen instead of employing high vacuum.

### Example 6

### Testing of block copolymers as timing layers

The polymer to be tested was coated from solution in methylethyl ketone (21.5 mg/dm²) above a hardened Lytron (trade Mark of G.A.F. for poly(styrene)co-(maleic anhydride)) layer (38 mg/dm²) on polyethylene-coated paper. The cover sheet, consisting of a layer of alizarin yellow indicator + gelatin coated on a polyethylene terephthalate film base, is soaked in 0.5 M KOH (20 secs.) and the two sheets laminated together, using hand rollers. The dye density was read by reflection every 1_{.}5 seconds, as the colour of the dye changed with changes of pH.

The timing layer breakdown time (TLB) was assessed as the time in seconds at which the density first begins to fall. The temperature coefficient is obtained from an Arhenius plot of measuring the release characteristics over a range of temperatures; the slope of a plot of log in °K gives the activation energy or, more precisely the temperature coefficient. Both properties are recorded in Table II below.

### Examples 7-11

Further block copolymers were prepared using the method of Examples 1-6 except that tetrahydrofuran (THF) was used in place of benzene in Examples 7-10. Experimental details and total polymer yield are given in Table III.

## Claims

1. A photographic colour diffusion transfer material containing an acid layer and a timing layer characterized in that the timing layer comprises an addition block copolymer comprising blocks of polymerised styrene or a substituted styrene and blocks of a homo- or co-polymer which is alkali-permeable or which becomes alkali-permeable after contact with alkali.

2. A photographic material as claimed in Claim 1 in which the styrene blocks are formed of polymerised styrene optionally substituted with an alkyl group containing 1-4 carbon atoms.

3. A photographic material as claimed in Claim 2 in which the styrene blocks are formed of polymerised styrene, p-methylstyrene or a-methylstyrene.

4. A photographic material as claimed in any of Claims 1-3 in which the alkali-permeable blocks are formed of a homo- or co-polymer containing acid groups or basic nitrogen-containing groups.

5. A photographic material as claimed in Claim 4 in which the alkali-permeable blocks are formed of polymerised vinyl acetate, N-vinylcaprolactam, N-vinylpyrrolidone, hydroxyethyl methacrylate, methacrylic acid or N-vinylimidazole either alone or in combination.

6. A photographic material as claimed in any of Claims 1-5 in which the block copolymer contains 10-45 weight percent styrene blocks.

7. A photographic material as claimed in any of Claims 1-5 in which the block copolymer contains 15-20 weight percent styrene blocks.

## Revendications

1. Produit pour la photographie en couleurs par diffusion transfert, contenant une couche acide et une couche retardatrice, caractérisé en ce que la couche retardatrice contient un copolymère d'addition séquencé comprenant des séquences de styrène ou de styrène substitué polymérisés et des séquences d'un homopolymère ou d'un copolymère qui est perméable aux alcalis ou qui le devient après contact avec un alcali.

2. Produit photographique, conforme à la revendication 1 dans lequel les séquences de styrène sont formées de styrène polymérisé, éventuellement substitué par un groupe alkyle contenant 1 à 4 atomes de carbone.

3. Produit photographique, conforme à la revendication 2 dans lequel les séquences de styrène sont formées de styrène de p-méthylstyrène ou de α-méthyIstvrène polymérisés.

4. Produit photographique, conforme à l'une quelconque des revendications 1 à 3, dans lequel les séquences perméables aux alcalis sont formées d'un homopolymère ou d'un copolymère contenant des groupes acides ou des groupes basiques contenant de l'azote.

5. Produit photographique, conforme à la revendication 5 dans lequel les séquences perméables aux alcalis sont formées des monomères polymérisés, seuls ou en combinaison, acétate de vinyle, N-vinylcaprolactame, N-vinylpyrrolidone, méthacrylate d'hydroxyéthyle, acide méthacrylique ou N-vinylimidazole.

6. Produit photographique, conforme à l'une quelconque des revendications 1 à 5, dans lequel le copolymère séquencé contient 10 à 45% en masse de séquences de styrène.

7. Produit photographique, conforme à l'une quelconque des revendications 1 à 5, dans lequel le copolymère séquencé contient 15 à 20% en masse de séquences de styrène.

## Patentansprüche

1. Fotografisches Farbdiffusionsübertragungsmaterial, das eine Säureschicht und eine Zeitsteuerschicht enthält, dadurch gekennzeichnet, daß die Zeitsteuerschicht ein Additionsblockcopolymer aufweist, das Blöcke aus polymerisiertem Styrol oder einem substituierten Styrol und Blöcke aus einem Homo- oder Copolymer enthält, das für Alkali durchlässig ist oder für Alkali durchlässig wird, wenn es mit diesem in Berührung gebracht wird.

2. Fotografisches Material nach Anspruch 1, dadurch gekennzeichnet, daß die Styrolblöcke aus gegebenenfalls mit einer Alkylgruppe mit 1-4 Kohlenstoffatomen substituiertem polymerisiertem Styrol bestehen.

3. Fotografisches Material nach Anspruch 2, dadurch gekennzeichnet, daß die Styrolblöcke aus polymerisiertem Styrol, p-Methylstyrol oder a-Methylstyroi bestehen.

4. Fotografisches Material nach einem der Ansprüche 1 bis 3, dadurch gekennzeichnet, daß die für Alkali durchlässigen Blöcke aus einem Homo- oder Copolymer mit Säuregruppen oder basischen stickstoffhaltigen Gruppen bestehen.

5. Fotografisches Material nach Anspruch 4, dadurch gekennzeichnet, daß die für Alkali durchlässigen Blöcke aus polymerisiertem Vinylacetat, N-Vinylcaprolactam, N-Vinylpyrrolidon, Hydroxy- äthylmethacrylat, Methacrylsäure oder N-Vinylimidazol bestehen, wobei diese Verbindungen entweder allein oder in einer Kombination in ihnen enthalten sind.

6. Fotografisches Material nach einem der Ansprüche 1 bis 5, dadurch gekennzeichnet, daß das Blockcopolymer 10-45 Gewichtsprozent Styrolblöcke enthält.

7. Fotografisches Material nach einem der Ansprüche 1 bis 5, dadurch gekennzeichnet, daß das Blockcopolymer 15-20 Gewichtsprozent Styrolblöcke enthält.
